

E. D. C. BAYNE & L. A. SUBERS.

REINFORCED COATED CORD OR THREAD.

APPLICATION FILED JAN. 21, 1908.

918,414.

Patented Apr. 13, 1909.



*Fig. 2*



Witnesses

A. S. Desbord  
J. B. Sawyer

Inventors

Eugene D.C. Bayne  
and Lawrence A. Subers  
by H. M. Monroe,  
Attorney

# UNITED STATES PATENT OFFICE.

EUGENE D. C. BAYNE AND LAWRENCE A. SUBERS, OF CLEVELAND, OHIO.

## REINFORCED COATED CORD OR THREAD.

No. 918,414.

Specification of Letters Patent. Patented April 13, 1909.

Application filed January 21, 1908. Serial No. 411,960.

To all whom it may concern:

Be it known that we, EUGENE D. C. BAYNE and LAWRENCE A. SUBERS, citizens of the United States, and residents of Cleveland, 5 county of Cuyahoga, State of Ohio, have invented certain new and useful Improvements in Reinforced Coated Cord or Thread the Component Strands of which are Coated, of which we hereby declare the following to 10 be a full, clear, and exact description, such as will enable others skilled in the art to which it appertains to make and use the same.

The objects of the invention are to provide 15 a cord or thread similar to the cord or thread described in our previous application for Letters Patent of the United States bearing Serial Number 380,401. This cord or thread was characterized by an exterior coating or 20 envelop of non-fibrous, tenacious and preferably vulcanizable material, and the cord or thread was composed of individual strands twisted together, each strand being separately coated with or enveloped in a similar 25 non-fibrous substance before twisting, whereby the strands in each cord or thread were maintained substantially out of contact with each other, and hence incapable of frictional 30 action upon each other, and also a series or group of such completed cords or threads, when afterward incorporated in a fabric, were separated by their exterior envelops, and would be incapable of frictional contact 35 with each other.

35 A fabric formed from strong fibrous material, such as flax, will possess great tensile strength, and on account of the enveloping coatings which prevent actual frictional contact of the fibers with each other will possess 40 a degree of flexibility impossible to obtain in any ordinary fabric.

This invention is designed to provide a cord or thread possessed of greater strength than the cord or thread shown and described in the said application, Serial Number 45 380,401, and also having a greater degree of durability and efficiency for many uses than the cord or thread of said application, without materially lessening the degree of 50 flexibility thereof or increasing its weight.

To accomplish these objects the previously coated fibrous strands are wrapped or twisted about a previously coated central reinforcing strand, and which remains perfectly 55 straight and is not twisted in with the other strands and its coating adheres strongly to

the coatings of the outer strands wrapped or twisted thereon.

The invention comprises therefore the central rectilinear coated strand and the exterior fibrous coated strands wrapped or twisted thereupon as hereinafter described and shown in the accompanying drawings and specifically pointed out in the claims.

In the accompanying drawings, Figure 1 65 is a view of a completed cord or thread, and Fig. 2 is a transverse section thereof.

In these drawings 1 represents the central reinforcing strand, 2, 2 the fibrous strands, 3, 3, the strand coatings, and 4 the external 70 coating.

It is important that the reinforcing strand or strands should be centrally located relative to the outer strands, so that it or they can not protrude or cut through the several envelops, and that the reinforcing strand shall be secured in place. Hence the fibrous strands must be wrapped or twisted closely about the reinforcing coated strand, so that it is tightly inclosed thereby, thus permitting 75 of flexible movement of the reinforcing strand in unison with the fibrous strands without injury to the envelops of the several strands or to the outer envelop of the thread, otherwise the reinforcing strand which is 80 preferably metal such as fine steel wire would soon cut its way through the non-fibrous material composing the several envelops.

The reinforcing strand can be formed 85 preferably of metal, such as steel, which can be annealed or tempered to any desired degree of hardness and flexibility, and made to sustain any desired degree of pressure or tension, compatible with its diameter. It is 90 preferable that the minimum tensile strength 95 of the metal strand should be at least equivalent to the maximum strength of all the fibrous strands.

A very strong fabric can be formed of this 100 material and if tubular can sustain a degree of internal pressure not possible in ordinary fabric, and the closeness with which such a fabric can be built up makes it durable and impenetrable to ordinary blows.

It is understood that in a fabric formed of 105 such cords or threads, the cords or threads are laid in each layer in parallel rows, their coatings adhering together, and the adjoining layers cross each other at an angle, thus obtaining tensile strength in at least two directions, similar to that shown and described 110 in our application for Letters Patent bear-

ing Serial Number 370,139. To obtain perfect smoothness in each layer of cords or threads, their exterior coatings should be compressed and formed into perfect cylindrical form.

5 We do not limit the kind of material employed in the central strand.

The central reinforcing strand can be a central strand of any material similarly 10 coated with a flexible and preferably vulcanizable material and adapted to increase the tensile strength of each cord or thread and being perfectly straight will lessen the tendency of the finished cord or thread to 15 stretch and assist in giving cohesion and shape thereto.

The strength of the finished cord or thread is greatly enhanced by the friction of the outer strands upon the central reinforcing 20 strand which opposes a strong resistance to any movement whatever of the outer strands thereon, such as would be caused by longitudinal strain, which would tend to elongate the spirally twisted or wrapped strands.

25 It is found that in this manner a practically non-extensible cord or thread is formed, that is, that can not stretch, since the addition of a relatively straight inner strand greatly increases the tensile strength of the 30 cord or thread and its value is commensurably greatly enhanced. As an illustration, a cord or thread of comparatively non-elastic fiber such as flax and of about one thirty second of an inch in diameter would have a 35 breaking or elastic limit of about twenty-five pounds. Then supposing a cord or thread to be composed of a specially prepared steel wire of approximately a sixty-fourth of an inch in diameter and four fibrous strands 40 are wrapped or twisted thereon having a sufficient diameter to bring the cord or thread up to a thirty second of an inch in diameter and the metallic strand to have a breaking or elastic limit of twenty pounds 45 and the fibrous strands to have a breaking limit of about eight pounds each, or a total of thirty two pounds, it will be seen that the collective strain sustainable by the finished cord or thread of one-thirty second of an 50 inch in diameter, would be in the neighborhood of fifty pounds.

The aggregate breaking strain of all the fibrous strands with which the central metallic strand is wrapped should preferably be 55 greater than that of the metallic strand, so as to enable all the strands to break in unison, since the fibrous strands are not twisted together but are wrapped or twisted about the metallic strand, hence they are not collectively as strong as if they were twisted together. However, if a fibrous central strand is employed the conditions are reversed. Since the breaking strain of the 60 central strand will be equal to or exceed that 65 of the several strands that envelop it.

The diameter of the reinforced cord or thread may be increased by increasing the diameters of the central and exterior strands and a stronger cord or thread obtained thereby.

70 When a fibrous central strand is employed, a cord or thread is increased about one-fifth in tensile strength over a cord or thread of the same diameter in which the central strand is not employed.

75 The relative thickness of the coatings upon the several strands and cord or thread can be determined by usage only. Since if too thick the strength of the fabric formed of the cords or threads is affected, and if not thick enough the vulcanizing process will practically obliterate it. It is sufficient if the coating substantially isolate the several strands and cords and threads so that they 80 are not in actual contact with each other.

85 Having described the invention what we claim as new and desire to secure by Letters Patent is:—

1. A thread comprising fibrous strands and a metallic strand grouped together, the 90 metallic strand being coated with an envelop of non-fibrous flexible material, and the fibrous strands being each saturated with and coated with an envelop of non-fibrous flexible material and the completed thread 95 also coated with a non-fibrous and flexible material, the said coatings upon said strands and threads being adhesive and vulcanizable.

2. A thread for an unwoven fabric comprising fibrous strands and a metallic strand 100 inclosed between the fibrous strands, said strands each coated with an envelop of non-fibrous and vulcanizable material, having a sticky surface prior to twisting and the completed thread provided with an exterior 105 coating of similar material.

3. A thread for an unwoven fabric, comprising a series of fibrous and a metallic strand united together, a separate coating upon each strand of non-fibrous and tenacious material and a similar coating upon the 110 completed thread.

4. A thread for an unwoven fabric, comprising a plural number of fibrous strands and a metallic strand, centrally inclosed between 115 the fibrous strands, each strand having a coating thereon of non-fibrous and adhesive material, the said strands adhering together to form the thread, and the completed thread having a coating of cylindrical and non-fibrous and adhesive material compressed 120 thereon.

5. A thread comprising fibrous strands and a metallic strand grouped together, the 125 said strands being each coated with a non-fibrous, flexible material, and the said completed thread also coated with a non-fibrous and flexible material, the said coatings upon said strands or threads being adhesive and vulcanizable and the said metallic strand and 130

its coating being inclosed by the said fibrous strands and their coatings.

6. A thread comprising fibrous strands, and a central reinforcing strand, the said fibrous strands being wound or twisted about and inclosing the said reinforcing strand, each of said strands being coated with a non-fibrous material, and the said completed thread being also coated with a non-fibrous and flexible material, the said coatings upon said strands and thread being adhesive and vulcanizable.

7. A cord or thread, comprising a central rectilinear untwisted reinforcing strand, and

a plurality of fibrous strands wrapped or 15 twisted closely about said central strand, each strand having a coating thereon of non-fibrous and adhesive material, and the finished cord or thread coated with a non-fibrous and adhesive material.

In testimony whereof we hereunto set our hands this 14th day of January, 1908, at Cleveland, Ohio.

EUGENE D. C. BAYNE.  
LAWRENCE A. SUBERS.

In presence of—

J. E. TAYLOR,  
A. T. OSBORN.